

# UNITED STATES PATENT OFFICE.

EDWARD LODGE AND JAMES MORGAN EVANS, OF HUDDERSFIELD, ENGLAND, ASSIGNEES TO LODGE-EVANS NEW YORK CORPORATION, OF NEW YORK, N. Y., A CORPORATION OF NEW YORK.

## PROCESS OF DYEING.

1,181,905.

Specification of Letters Patent.

Patented May 2, 1916.

No Drawing.

Application filed December 26, 1914. Serial No. 879,210.

To all whom it may concern:

Be it known that we, EDWARD LODGE and JAMES MORGAN EVANS, both subjects of the King of Great Britain, and residing at 5 Huddersfield, in the county of York, England, have invented a new and useful Improvement in Processes of Dyeing, of which the following is a specification.

Our invention relates to the application 10 of sulfur dye-stuffs for dyeing animal textile fibers and fabrics, (wool, hair, feathers, furs and silks) also artificial silks, and union goods composed of a mixture of animal and vegetable fibers and artificial silks, 15 (i. e., animal fibers, mixed with cotton, flax, jute, rhea, ramie, china grass or hemp).

The usual manner of applying sulfur colors to vegetable fibers and fabrics is to reduce and dissolve the color with the aid of 20 sodium sulfid. This method is however not applicable for dyeing animal fibers or fabrics containing animal fibers, owing to the strong alkalinity of the bath dye-liquors.

The applicants have found that, if the 25 sulfur colors be reduced to their leuco-compounds by means of a sulfid of an alkali-metal in presence of a normal sulfite of an alkali-metal, e. g.,  $Na_2SO_3$  or  $K_2SO_3$ , and the excess of sodium or potassium alkali removed, or exchanged for the weaker alkali, ammonia, animal fibers can thereby be dyed 30 without injury.

The action of the normal sulfite of an alkali-metal appears to be at least two fold. 35 It converts any free sulfur present in the color into thiosulfates and changes any polysulfids into thiosulfates and normal sulfids and secondly it dissolves (renders soluble) the coloring matter itself.

40 The dye bath is most conveniently prepared by first boiling together the color and sulfite of sodium or potassium, and water, then adding sulfid of sodium and stirring carefully until reduction and solution are 45 complete.

The sodium or potassium sulfid reacts with water to give the caustic alkali, sodium or potassium hydroxid, and the correspond-

ing hydrosulfid. These reactions may be expressed by the following equations:— 50



This concentrated solution of the prepared dye is added to the dye bath, containing the requisite quantity of water which has previously been heated to the required temperature and to which the neutral ammonium salt has been added. 55

Suitable ammonium salts are the chlorid, 60 normal sulfate and acetate.

When a solution of sodium or potassium is treated with an ammonium salt, the sodium or potassium is converted into the neutral salt of these metals and free ammonia is liberated, as expressed by the following 65 equations:—



In this way the powerful caustic alkalis, sodium and potassium hydroxids and hydrosulfids, are exchanged for the mild alkali ammonia. 75

The following is an example of a typical dye-bath prepared according to our invention from a commercial sulfur dye-stuff: To each liter of solution are added 5 grams concentrated sulfur dye, 10 grams sodium sulfite, 5 grams anhydrous sodium sulfid, 10 grams normal ammonium sulfate. 80

The temperature of the bath is varied according to the materials to be dyed. For wool, or the wool part of union goods a 85 temperature of  $70^{\circ}$ - $80^{\circ}$  C. is serviceable; for artificial silk and the cotton part of union goods a lower temperature will suffice.

As an example wool will be worked in 90 the dye solution at  $70^{\circ}$ - $80^{\circ}$  C. For unions of cotton and wool the cotton may be dyed at a temperature up to about  $40^{\circ}$  C. on raising the temperature up to  $70^{\circ}$ - $80^{\circ}$  the wool is then dyed. Or the order may be 95 reversed. The addition of Glauber's salt or

common salt assists, as is well known, exhaustion of the dye liquor.

What we claim is:

A method or process of dyeing animal fibers (including furs and feathers) union goods and artificial silk in any stage of manufacture, in which sulfur colors are reduced by a sulfid of an alkali - metal in

presence of a sulfite of an alkali metal and a neutral ammonium salt is added to the bath substantially as described.

EDWARD LODGE.

JAMES MORGAN EVANS.

Witnesses:

Wm. RAMSDEN,  
ARNOLD MELLOR.